

N. V. HYBINETTE.

PROCESS OF ELECTROLYTIC PRODUCTION OF COPPER.  
APPLICATION FILED MAR. 29, 1913.

1,084,150.

Patented Jan. 13, 1914.



Witnesses  
B. Dommers  
C. Leekert.

Inventor  
Noak Victor Hybinette  
J. Henry Orthofer

444

# UNITED STATES PATENT OFFICE.

NOAK VICTOR HYBINETTE, OF CHRISTIANIA, NORWAY.

## PROCESS OF ELECTROLYTIC PRODUCTION OF COPPER.

1,084,150.

Specification of Letters Patent.

Patented Jan. 13, 1914:

Application filed March 29, 1913. Serial No. 757,583.

To all whom it may concern:

Be it known that I, NOAK VICTOR HYBINETTE, a subject of the King of Norway, residing at Christiania, Norway, have invented certain new and useful Improvements in Processes of Electrolytic Production of Copper; and I do hereby declare the following to be a full, clear, and exact description of the invention, such as will enable others skilled in the art to which it appertains to make and use the same.

In processes where copper is produced direct from ores by leaching and electrolysis there is generally present in the electrolyte large quantities of iron, which make the electrolytic deposition of the copper impossible. The trouble shows itself by dissolving the deposited copper at the top of the cathode plate while some deposition is going on at the bottom part of the same cathode. The cathode plate is finally entirely dissolved or eaten away at the upper part, and the remainder falls to the bottom of the tank. Theoretically this is explained by the fact that the ferric sulfate in the electrolyte acts upon the copper at the cathode to form ferrous sulfate which is oxidized at the anode to the ferric form and again passes to the cathode to dissolve more copper.

In processes heretofore used it is specified that the presence of ferric compounds at the cathode should be avoided, and this has been accomplished by reducing the solution with ore to such an extent, as the nature of the ore permits, and then completing the reduction with sulfuric acid gas before passing the solution to the cathode. In connection herewith the cell in which the plating has taken place for the same reason has been constructed with a very tight diaphragm so as to prevent the ferric salts formed at the anode from entering the cathode compartment. The above practice resulted in the production of sulfuric acid from the  $\text{SO}_2$ , and the too strongly acid solution dissolved undue proportions of iron and other impurities, which made it necessary to frequently renew the electrolyte.

The object of my invention is a process worked out on the basis of a new principle or theory, whereby the process may be carried out in a more advantageous manner.

When copper is electrolytically deposited from a solution containing copper and iron salts with the aid of an insoluble anode, the

iron salts are oxidized at the anode. This oxidizing not only causes the formation of ferric salts, but also higher oxidation compounds of iron, which, however, are easily decomposed by the ferrous salts present in excess of the electrolysis. Supposing now that these higher oxidized compounds have the formula  $\text{Fe}_2\text{O}_5$ , the composition of the solution at the anode may be indicated by the formula:



The first and the last of these compounds will in a short time react with the other so as to form  $\text{Fe}_2\text{O}_3(\text{SO}_4)_3$ , as follows:



If now the solution circulates in such a way that it becomes possible for some of the solution at the anode to reach the cathode before sufficient time has elapsed to allow the higher compounds to be reduced by the ferrous salts present in excess in the electrolyte, then metallic copper is dissolved, and this explains the fact that the same cathode can be dissolved at its upper portion and have copper deposited simultaneously on its bottom portion.

The main feature of my process consists therefore, in that the cathode is separated from the anode by a very porous diaphragm or filter, and in causing the solution coming from the leaching tanks and containing considerable quantities of ferric salts to enter the cell at the cathode, and thereupon be allowed to filter through said diaphragm into the anode compartment. By this method the ferric salts in the anode compartment are prevented from returning to the cathodes. In this way it is possible to avoid the reduction of the cathode solution by the necessity of sulfuric acid, as well as the drawbacks resulting from such reduction, and at the same time it is possible to obtain better results in the way of more complete extraction when a higher percentage of ferric salts is present in the solution.

According to my experience the process may be carried out with a solution going to the cathode cell containing, per liter, 20-30 grains of iron in the form of ferric salts ( $\text{Fe}_2\text{O}_3$ ). When ferric salts are present at the cathode there is a reduction of the amount of copper deposited, but this re-

duction is not so great as to make the process uneconomical, and as the deposition takes place evenly all over the surface of the cathode, there is no practical hindrance 5 in carrying out the process. The reduction of ferric salts to ferrous salts, which it is necessary to accomplish before the copper will be deposited upon the cathode is, therefore, in my process effected by the electric 10 current, and a certain amount of electric energy is consumed for the purpose, but only so much reduction is effected as is necessary, and I avoid the complete reduction and the introduction of sulfuric acid, 15 which has proven itself so harmful in other processes.

It has heretofore been supposed, that no copper will be deposited before all ferric salts are reduced, but I have found that 10 20 to 15 grams of iron can easily be present in the ferric state without materially affecting the efficiency as regards the amount of copper plated, provided, however that care is taken, that fresh solution from the 25 anode is not allowed to pass to the cathode.

I have constructed a diaphragm especially adapted for this process, which diaphragm consists of a very porous material such as loose cotton or asbestos held in place 30 or strengthened by means of a metallic (leaden) skeleton. This diaphragm is the subject matter of my Patent No. 1,052,256 dated February 14, 1913. By the use of a filtering partition, instead of a diaphragm 35 in the usual meaning of the word, I have less resistance, and therefore also less power consumption. The disadvantage of having a mechanically weak diaphragm has been overcome by the use of the said lead construction, which supports the soft fibrous 40 material of the diaphragm.

The accompanying drawing shows a vertical section through an electrolytic cell consisting of a tank A in which the anodes 45 B are suspended on each side of the cathode chamber built up of a framework K and filtering partitions D, between which is placed the cathode C. The solution enters at H, passes through the partitions D and 50 out at G. It is evident that not the whole of the solution need circulate through the filter or diaphragm, and that I may supply only enough solution into the cathode com-

partment to keep up the desired concentration of copper, and there is nothing to prevent another quantity of solution from being circulated in the anode compartment only, for the purpose of oxidizing the iron prior to leaching fresh quantities of ore. By such circulation, I am able to obtain a 60 better oxidizing efficiency at the anode than if the circulations were limited to the small amount filtering through the diaphragms. 65

By means of this process poor copper ores with a large content of iron may also with 70 advantage be treated electrolytically. Owing to the fact that no sulfurous acid is used, the solution can be maintained at a comparatively low degree of acidity, and this makes it possible to carry out the leaching 75 operation with solutions after being depleted of copper without dissolving too large quantities of iron. A solution such as that employed in this process has also the advantage of having a great dissolving power, not only upon copper compounds that are soluble in sulfuric acid, but also upon copper in other forms, such as sulfid of copper and metallic copper.

The employment of a filter-like dia- 80 phragm constructed as above described facilitates the working of the process, as the diaphragm may be easily cleansed, and also easily and in an inexpensive manner renewed. The employment of leaden structures has proved to be connected with no 85 drawbacks. The utilization of this property of lead is one of the important features of this invention.

I claim—

The process of electrolytic production of copper by leaching of ore and plating from a solution containing both copper and iron salts, which comprises passing an electrolyte containing large quantities of ferric 95 salts into the cathode compartment of an electrolytic cell and circulating the solution through a filter in direction from cathode to anode.

In testimony that I claim the foregoing 100 as my invention, I have signed my name in presence of two subscribing witnesses.

NOAK VICTOR HYBINETTE.

Witnesses:

M. E. GUTTORMSEN,  
RUTH LINDSTRÖM.